

1,375,826.

L. CAMMEN,  
CASTING METAL TUBING.  
APPLICATION FILED JAN. 24, 1921.

Patented Apr. 26, 1921.



Fig. 1



Fig. 2



Fig. 3

INVENTOR.

Leon Cammen  
BY  
L. Cammen

# UNITED STATES PATENT OFFICE.

LEON CAMMEN, OF NEW YORK, N. Y.

## CASTING METAL TUBING.

1,375,826.

Specification of Letters Patent. Patented Apr. 26, 1921.

Application filed January 24, 1921. Serial No. 439,574.

To all whom it may concern:

Be it known that I, LEON CAMMEN, a citizen of the United States, and resident of borough of Manhattan, in the city, county, 5 and State of New York, have invented certain new and useful Improvements in Casting Metal Tubing, of which the following is a specification.

This invention refers to the production 10 by centrifugal casting of tubing from metals having a high melting point and such that overheating previous to casting is not desirable. Such is for example Monel metal which has a melting point in the proximity 15 of 2500 deg. F., and which loses some of its copper content if heated considerably beyond its melting point.

When such metal is cast centrifugally by the usual processes (melting the metal in a 20 crucible and pouring it into a cold mold), it chills long before it has had time to form a pipe, which is the reason why no Monel metal tubing has been hitherto produced.

The present invention describes a method 25 of procedure by which the above difficulties are successfully overcome.

In the illustrations,

Figure 1 is a cross-section of the mold 30 normal to the axis of spinning; Fig. 2 is a view from on-top of part of the mold along a section along the axis of rotation;

Fig. 3 is a sectional view of the same 35 mold, including a metal rod from which a tube is to be made.

Essentially, the present invention involves the use of a mold of such construction that the part which comes in contact with the metal, could be heated to such a temperature that the metal would remain fluid 40 when coming into contact with it, and yet the entire mold would remain sufficiently strong mechanically to be used for centrifugal spinning.

Assuming that it is desired to make tubing 45 of such material as Monel metal, this latter has to be poured into the mold at a temperature which cannot be lower than say 2480 deg. F. (theoretical melting temperature of Monel metal), and not higher than 50 say 2600 deg. F., as experience has shown that above that temperature the Monel metal begins to lose its copper.

It is obvious therefore that the lining of 55 the mold into which the metal is poured, must have a temperature in the region of

2000 deg. F. (white heat for graphite), in order to permit the metal to stay hot long enough to complete the process of spinning. These figures are based on the general experience in founding Monel metal, and on 60 my own tests.

On the other hand, however, Monel metal tubing has to be cast in lengths of 12 to 20 feet, and diameters varying from  $\frac{1}{2}$  inch 65 up. It is obvious to any person who has had experience in foundry work that it is impossible to heat a lining 12 to 20 ft. long, and of a small inside diameter, by shooting a flame, such as a gas flame, through it, as 70 only the ends will be heated in this manner. The other, and simpler, way, viz., to heat the pipe together with the lining to a white heat, is entirely out of the question, as steel pipe heated to white heat would be so 75 weak mechanically that the lining would buckle and crack as soon as the spinning started.

To obviate these difficulties, the present 80 invention provides a process of casting by centrifugal spinning in which use is made of a composite mold, such as is shown in Fig. 1, and the lining is heated electrically. In Fig. 1, 1 is a conducting (electrically) 85 lining, such as graphite; 2 is a body acting as an electrical insulator, thus confining the flow of current to the lining 1, and keeping it away from the metal pipe 3, and finally this latter pipe 3, the purpose of which is to give mechanical strength to the mold. 90

The current may be introduced into the lining 1, as shown in Fig. 2, by heavy copper or steel rings 4 and 5 (which may be water cooled in the usual manner if desired), connected by leads 6 and 7 with a source of electric current, such as the secondary of a transformer 8 (primary not shown). 95

The intermediary body 2 should be preferably selected in such a manner as to be a poor conductor both electrically and thermally, under which conditions the lining 1 may be brought to a white heat, while the metal pipe 3 remains comparatively cool. 100

Fig. 3 shows one more step in the application of the same principle. The graphite lining 1 is closed by carbon blocks 11 and 10 insulated from the pipe 3 by the intermediary body 2, and a rod 12 of the metal from which the pipe is to be made is held between the end blocks 9 and 10, current being supplied to these latter by the leads 6 and 7 105 in the same manner as in Fig. 2. 110

As the conductivity of the metal rod is very much superior to that of the graphite lining, the main current will go through the rod. Enough current however will go

- 5 through the lining to make it hot, which is also assisted by the radiation from the rod. In order to keep the lining uniformly hot, it is advisable to rotate the mold slightly, as by pulley 13, and belt (not shown) during the process of melting of the rod, which is especially advisable toward the end of the process of melting when the rod sags, and if stationary, is apt to overheat one section of the lining, and cause subsequent 15 cracking.

No claims are made for the mold itself, as this will form the subject of a separate application.

I claim:

- 20 1. A process of manufacture of metal tubing by centrifugal casting, wherein is used a composite mold, consisting of not less than three parts, such that part one which comes in contact with the metal of the tube, is electro-conductive; part two, essentially surrounding part one, is electro-insulative, and part three is of metal; and wherein further the lining, which is part one of the mold, is heated, previous to the 25 pouring of the metal, by an electric current to a temperature close to the melting point of the metal.

2. A process of manufacture of metal tubing by centrifugal casting wherein is 30 used a composite mold consisting of not less than three parts, such that part one which comes in contact with the metal of the tube is electro-conductive; part two essentially surrounding part one, is electro-insulative, 35 and part three is of metal; and wherein

further the metal of the tube is heated to the melting point by the passage of the electric current previous to the start of centrifugal spinning.

3. A process of manufacture of metal 45 tubing by centrifugal casting wherein is used a composite mold consisting of not less than three parts, such that part one which comes in contact with the metal of the tube is electro-conductive; part two essentially surrounding part one, is electro-insulative, and part three is of metal, and wherein further the metal of the tube is heated to the melting point by the passage of an electric current previous to the start of the centrifugal spinning, but during the heating of the metal of the tube the mold is subjected to a rotation at a speed below that used for centrifugal spinning.

4. A process of manufacture of metal 50 tubing by centrifugal casting wherein the metal of the tube is heated to the melting point by the passage of an electric current in the same mold in which it is subjected to the spinning process.

5. A process of manufacture of metal tubing by centrifugal casting wherein the metal of the tube is heated to the melting point by the passage of an electric current 55 in the same mold in which it is subjected to the spinning process, the mold, during the heating of the metal, being rotated at a speed below that used for centrifugal spinning.

Signed at New York, in the county and 75 State of New York, this 19 day of January, 1921.

LEON CAMMEN.

Witness:

C. C. CAMMEN.